

## UNITED STATES PATENT OFFICE

OTHO V. STEWART, OF WILKINSBURG, PENNSYLVANIA, ASSIGNOR TO WESTINGHOUSE ELECTRIC & MANUFACTURING COMPANY, A CORPORATION OF PENNSYLVANIA

## POLISHING COMPOUND

No Drawing.

Application filed December 8, 1925. Serial No. 74,192.

My invention relates to a composition of matter, and especially to a compound for polishing and varnishing extremely hard materials.

5 It is one of the objects of my invention to provide a polishing compound containing a material that shall remove imperfections in the surfaces of extremely hard materials and which has properties that render it valuable 10 for producing burnished surfaces on said materials.

A polishing compound must possess the properties of an abrasive or cutting material to the extent that imperfections in the 15 surface of the material that is being polished are rapidly removed and, at the same time, it must have a definite lubricating property that prevents the abrasive from rapidly cutting the smoothed surface of the material 20 after the imperfections are removed.

I have discovered an improved polishing compound that is suitable for polishing the surfaces of extremely hard materials, particularly the surface of chromium metal. When 25 my compound is utilized in a hand-polishing operation, or on a centrifugal buffer wheel, the material operates to cut away small raised portions and imperfections in the surface of the metal, but it does not possess sufficient cutting power to continue rapid abrading 30 of a relatively smooth surface.

My improved polishing compound is a mixture of green chromic oxide ( $Cr_2O_3$ ) and stearine wax, mixed in the proportions of 35 about two parts oxide to about 1 part stearine wax. The chromic oxide is prepared by reducing it to a fine powder containing particles insufficient in size to produce visible scratches in the polished surface. The oxide may be 40 reduced to such degree of fineness by grinding, or by any of the other well-known methods.

The oxide and the stearine wax are mixed in the above-noted proportions as follows: 45 The wax is heated to 90° to 100° C. and the chromic oxide is slowly stirred into the wax in such manner that a smooth paste results. The mixture may then be poured into molds to cool.

0 I may vary the properties of the mixture

by adding a small amount of a light hydrocarbon oil, such as kerosene. The light oil provides a softening effect on the compound according to the amount used and it provides a polishing compound having slightly better lubricating properties than the wax-oxide composition. I may use an amount of kerosene equal to 1 to 10% of the weight of the wax. A preferred composition is made by adding about 1% kerosene oil to the mixture 55 of oxide and wax.

Although I have described a preferred composition and a modification thereof, I may utilize a light lubricating oil instead of kerosene, or I may still further modify the 65 compound by substituting another wax-like lubricant provided the lubricant retains the oxide in suspension and preserves an even distribution of oxide throughout the finished compound. Other modifications of my invention will suggest themselves to those skilled in the art without departing from the spirit of 70 my invention, as defined in the annexed claims.

I claim as my invention:

1. A composition of matter which consists of finely divided green chromic oxide intimately mixed with stearine wax.

2. A composition of matter which consists of finely divided green chromic oxide intimately mixed with a vehicle having lubricating properties.

3. A composition of matter which consists of finely divided green chromic oxide intimately mixed with a vehicle having lubricating properties and being capable of retaining a constant distribution of said oxide throughout said vehicle.

4. A composition of matter which consists of finely divided green chromic oxide intimately mixed with stearine wax in the proportions of about 1 part stearine wax to 2 parts oxide.

5. A composition of matter which consists of finely divided green chromic oxide intimately mixed with a vehicle having lubricating properties and a small amount of a light hydrocarbon oil.

6. A composition of matter which consists of finely divided green chromic oxide in-

75

80

85

90

95

100

timately mixed with a vehicle having lubricating properties and a small amount of kerosene oil.

In testimony whereof, I have hereunto subscribed my name this first day of December,  
**5** 1925.

**OTHO V. STEWART.**

**10****15****20****25****30****35****40****45****50****55****60****65**